

## 1

3,232,718

### ELECTROCHEMICAL PRODUCT

Edgar J. Seyb, Jr., Oak Park, and Augustine J. Wallace, Jr., East Detroit, Mich., assignors to M & T Chemicals Inc., New York, N.Y., a corporation of Delaware

No Drawing. Original application June 17, 1960, Ser. No. 36,750, now Patent No. 3,141,836, dated July 21, 1964. Divided and this application July 31, 1963, Ser. No. 306,646

#### 1 Claim. (Cl. 29—194)

This application is a division of our application Serial No. 36,750 filed June 17, 1960, now Patent 3,141,836.

The present invention is directed to improved baths and process for electroplating tin-nickel alloys and to bright tin-nickel electrodeposits.

Plating baths for electrodepositing tin-nickel have ex-

## 2

lustrous. We have been able to increase brightness to (i) hazy-bright, a slight background, haze in an essentially clear deposit, and (ii) clear-bright, brightness approaching that normally associated with a mirror. By using the various additives specified hereinafter, it is possible to obtain hazy-bright and/or clear-bright deposits. These deposits are lustrous. Lustrous and bright deposits are obtained from acid baths containing, as a brightener, phenylpropionic acid; phenylpropionic amide; triaminotriphenyl methane; 1-(p-aminophenyl)-3-methylpyrazole; stearamidopropyldimethyl - ( $\beta$ -hydroxyethyl)ammonium dihydrogen phosphate; or 1,5-diphenylcarbohydrazide.

These bright deposits are physically different from any heretofore produced. They apparently have a finger-grained structure. They differ appreciably in the grain orientation with strong layering in the 300 plane. X-ray diffraction data follows:

TABLE I

| Published X-ray data |                  |                 | Observed intensity |              |              |
|----------------------|------------------|-----------------|--------------------|--------------|--------------|
| d/n                  | (Plane)<br>h k l | A—No brightener | B—No brightener    | C—Brightener | D—Brightener |
| 2.94                 | 101              | s               | m                  | -----        | -----        |
| 2.076                | { 102<br>110     | vs              | s                  | vw           | w            |
| 1.198                | 300              | m               | m                  | vs           | s            |

cellent throwing power. Although the electrodeposits obtained from commercial baths are fairly attractive, the deposits are not as clear and bright as required for most decorative applications. Only those deposits plated over a bright undercoat in thicknesses less than 6 microns "appear" bright. Essentially here the deposit is transparent. In thicknesses greater than 6 microns, there is a slight white clouding-over of the deposit resulting in a hazy deposit, which increases with increased thickness. It is desirable to have a clear, lustrous deposit and even more desirable to have a clear, bright deposit. We have now discovered a process utilizing special baths from which we are able to electrodeposit bright tin-nickel.

It is an object of this invention to provide lustrous tin-nickel alloy electrodeposits.

It is also an object of this invention to provide bright tin-nickel electrodeposits in thicknesses greater than 6 microns.

The invention also contemplates improved baths electrodepositing lustrous, clear and bright tin-nickel alloys in thicknesses greater than 6 microns.

The invention further contemplates a process for electrodepositing lustrous, clear, and bright tin-nickel electrodeposits in thicknesses greater than 6 microns.

We discovered that lustrous and bright tin-nickel electrodeposits may be obtained from acidic baths which contain an effective amount of a brightener. We discovered that specific compounds and combinations of specific compounds are effective brighteners for tin-nickel alloy electrodeposition.

The electrodeposit may be made on dull basis metals, although this is not preferred. As deposited initially, the tin-nickel is fairly bright and as electrodeposition continues, the deposit becomes increasingly bright resulting in a lustrous deposit. Tin-nickel as electrodeposited from standard baths may be described as "cloudy-bright." The deposit has a slight white clouded appearance. It is not

30 The designation of the intensity of the lines is as follows:

vs—very strong

s—strong

m—medium

w—weak

vw—very weak

40 The data for the deposit noted in Column A is reproduced from J. of Electrodepositors' Tech. Soc., 27, 156 (1950-51), as is the d/n and h k l values. The data in Column B is for a deposit obtained from Bath No. 2 of Table II herein, using the potassium salt of perfluoroethylcyclohexane sulfonate as an anti-pitting agent. The bright deposits recorded in Column C and Column D were from the same bath as that of Column B; the bath of Column C also containing 0.2 g./l. of phenylpropionic acid as a brightener; and that of Column D containing 0.2 g./l. of stearamidopropyldimethyl - ( $\beta$ -hydroxyethyl)ammonium dihydrogen phosphate as a brightener. The deposits of 50 Columns B, C, and D were 0.015 cm. thick.

55 Phenylpropionic acid, phenylpropionic amide, and triaminotriphenyl methane are useful brighteners when added to the baths in amounts between 0.01 g./l. and 0.3 g./l.; preferably baths containing 0.05 g./l. and 0.2 g./l. are used. 1-(p-aminophenyl)-3-methylpyrazole is a useful brightener when added to the bath in amounts between 0.05 g./l. and 1 g./l.; preferably baths containing 0.2 g./l. and 0.5 g./l. are used. Stearamidopropyldimethyl - ( $\beta$ -hydroxyethyl)ammonium dihydrogen phosphate is a useful brightener when added to the bath in amounts between 0.001 g./l. and 0.2 g./l.; preferably baths containing 0.01 g./l. and 0.1 g./l. are used. 1,5-diphenylcarbohydrazide is a useful brightener when added to the bath in amounts between 0.05 g./l. and 0.5 g./l.; preferably baths containing 0.2 g./l. and 0.3 g./l. are used.

When one of the aforementioned brighteners is used as the sole brightener in the bath, effective brightening action is not achieved when the bath contains less than the minimum concentration specified for each brightener. Smaller concentrations may be extremely effective when more than one brightener is used in combination. The maximum preferred concentration specified for each brightener is that concentration at which acceptable brightness will be achieved with the variation of conditions to be found in commercial practice. Above the preferred maximum concentration specified, the deposit tends to become brittle at high current densities (above about 7.5 amp./sq. dm.). Above the maximum concentration specified, the brittleness becomes severe enough to cause cracking and some exfoliation so that the current density range is substantially reduced.

Phosphoric acid and its salts have also been discovered to be brighteners. Phosphoric acid when added to the bath in amounts between 0.1 g./l. and 15 g./l., and preferably between 0.5 g./l. and 7 g./l., results in lustrous, hazy-bright deposits. The brightness activity is most significant in the 0.5-7.0 g./l. range. Although amounts in excess of 7.0 g./l. up to 15 g./l. do not appear to produce an increase in the brightness of the deposit, this presence does not give detrimental effects. Above about 15 g./l., the deposit possesses a grainy appearance. Concentrations of less than 0.5 g./l. are effective when used in combination with a sufficient concentration of another brightener. Phosphoric acid as used herein includes the ortho, pyro, meta- and hypo-phosphoric acid as well as the equivalent series of salts. The potassium, sodium, and ammonium salts are preferred.

Combinations of the various brighteners give unusually good deposits; in particular, deposits approaching mirror-brightness have been obtained by using phosphoric acid in combination with one of the other brighteners. Although the ranges in which the individual brighteners are effective are also the same general ranges in which they are effective in combination, it is possible to use amounts smaller than the minimum specified concentration of one brightener, in combination with another brightener in relatively higher concentrations. The combinations of brighteners are particularly preferred in that the brightest deposits are obtained with combinations of brighteners. The use of phosphoric acid in combination with one of the other brighteners has been particularly useful in that it tends to broaden the limits of the range of concentrations of brightener permitted in the bath. A preferred method of incorporating the brightener in the bath is to add a water solution containing 5 g./l. to 200 g./l. of phosphoric acid and 5 g./l. to 50 g./l. of at least one of the other brighteners specified herein.

Tin-nickel is deposited from acid baths, primarily from chloride and/or fluoride baths. The preferred baths contain both chloride and fluoride anions, stannous tin in the amounts of 26 g./l. to 37.5 g./l.; and nickel in amounts between 60 g./l. and 82.5 g./l. The total fluorine for new baths is between 34 g./l. and 45 g./l. in the mixed baths. The stannic tin concentration increases in baths which are in operation. As this occurs, the fluorine should be increased so that it at least equals the total tin in the bath. The chloride content is not critical. The pH is maintained between 2 and 3.5, generally by the addition of ammonium hydroxide or hydrofluoric acid. To prevent pitting, the baths should also contain a suitable agent. A class of agents which has been found to be satisfactory includes a sulfonated cyclic fluorocarbon such as perfluoro-4-methyl cyclohexyl sulfonic acid; perfluorocyclohexyl sulfonic acid; perfluoro-2-methyl cyclohexyl sulfonic acid; perfluoro-1-methyl cyclohexyl sulfonic acid; perfluoro-2,5-dimethyl cyclohexyl sulfonic acid; perfluoro-4-ethyl cyclohexyl sulfonic acid; perfluoro-4-isopropyl cyclohexyl sulfonic acid; and the salts of these acids. The bath is

operated at high temperatures, preferably between 65° and 71° C. Typical bath formulations follow:

TABLE II

|    | Bath 1:                                                          | Grams per liter |
|----|------------------------------------------------------------------|-----------------|
| 5  | Stannous chloride, $\text{SnCl}_2$ -----                         | 42              |
|    | (Tin metal) -----                                                | 26              |
| 10 | Nickel chloride, $\text{NiCl}_2 \cdot 6\text{H}_2\text{O}$ ----- | 300             |
|    | (Nickel metal) -----                                             | 75              |
| 15 | Sodium fluoride, $\text{NaF}$ -----                              | 28              |
|    | (Fluoride) -----                                                 | 13              |
| 20 | Ammonium bifluoride, $\text{NH}_4\text{HF}_2$ -----              | 35              |
|    | (Fluorine) -----                                                 | 24              |
| 25 | Total fluorine in bath -----                                     | 37              |
|    | pH (colorimetric), 2.5                                           |                 |
| 30 | Temperature, 65° C.                                              |                 |
| 35 | Cathode current density, 3 amp./sq. dm.                          |                 |

|    | Bath 2:                                                             | Grams per liter |
|----|---------------------------------------------------------------------|-----------------|
| 20 | Stannous chloride -----                                             | 49              |
| 25 | Nickel chloride ( $\text{NiCl}_2 \cdot 6\text{H}_2\text{O}$ ) ----- | 300             |
| 30 | Ammonium bifluoride ( $\text{NH}_4\text{HF}_2$ ) -----              | 56              |
| 35 | Ammonium hydroxide, as needed to adjust pH to 2.0-2.5               |                 |
| 40 | Temperature, 68° C.                                                 |                 |

All-chloride baths are generally operated at lower pH's, i.e., not greater than about 1, by the addition of hydrochloric acid. In these all-chloride baths, the tin is added in the form of stannous chloride, and the nickel in the form of nickel chloride. All of the baths are initially made up by adding the noted chemicals to water. However, equivalent chemicals may be added, e.g., stannous tin may be added in the form of the oxide or the fluoride, as well as the chloride. During operation, the tin and nickel may be replaced either chemically or by anodic corrosion of metallic anodes or a combination of both.

For the purpose of giving those skilled in the art a better understanding of the invention, the following illustrative examples are given. In the examples, tin-nickel (approximately 65% tin and 35% nickel) was electro-deposited at the conditions noted. The physical appearance of the deposit obtained in each example is described. As noted they are lustrous and bright and in some cases they are a clear-bright.

45 All the samples were plated from the standard bath identified as Bath 2 of Table II hereinbefore. Plating tests were made under two different sets of conditions as specifically noted in each example. Most of the test cathodes were plated in a "Hull Cell" which is described on pages 645-648 of The Metal Finishing Guidebook, 27th Edition (1959). With this procedure, the current density changed along the length of the panel so that the appearance of a deposit could be examined over a current density range of about 0.5 to 8 amperes per square decimeter. In the 50 other tests, small zinc die cast handles were used. This showed the tin-nickel deposit as it would appear on a production part. When the zinc part was used, the plating was done in a small laboratory tank rather than in a Hull Cell. In both instances, mild solution agitation was used.

#### Example 1

55 Triaminotriphenyl methane was added to the standard bath in the amount of 0.25 g./l. Under the standard plating conditions, a small copper plated zinc die cast handle was plated at an average current density of approximately 2.3 amperes per square decimeter (amp./sq. dm.) for 25 minutes to an average thickness of approximately 20 microns. The deposit was clear-bright over the decorative area of the handle to give a lustrous, attractive article.

#### Example 2

60 Triaminotriphenyl methane in the amount of 0.05 g./l. was added to the standard bath which was placed in a Hull Cell. In this plating cell, a smooth brass panel was

plated as cathode for 10 minutes with the current adjusted so that the current density ranged from a low of approximately 0.05 amp./sq. dm. at one end of the panel to about 8 amp./sq. dm. at the other end of the panel. The average thickness of the tin-nickel was approximately 9 microns and the thickness at the high current density end of the panel was approximately 27 microns. The deposit was hazy-bright in appearance over the entire panel.

*Example 3*

Phenylpropionic acid in the amount of 0.2 g./l. was added to the standard bath in a small plating tank. Tin-nickel was plated directly on a steel cathode at an average current density of 2.3 amp./sq. dm. for 45 minutes to give an average thickness of approximately 40 microns. At this thickness a hazy-bright deposit was obtained over the surface of the cathode.

*Example 4*

Phenylpropionic acid in the amount of 0.14 g./l. was added to the standard bath formulation and placed in a Hull Cell. A smooth brass panel was plated in this cell at an average current density of 2.7 amp./sq. dm. for 10 minutes. Over the current density range of 0.05 to 8 amp./sq. dm. the deposit was clear-bright and lustrous.

*Example 5*

Phenylpropionic acid in the amount of 0.04 g./l. was added to the standard bath formulation in a Hull Cell. With a smooth brass panel as cathode plated at 2.7 amp./sq. dm. for 10 minutes, the deposit was hazy-bright.

*Example 6*

Phenylpropionic amide in the amount of 0.25 g./l. was added to the standard tin-nickel bath in a Hull Cell. A smooth brass panel was plated at an average current density of 2.7 amp./sq. dm. for ten minutes. At the end of this time the plate was clear-bright and lustrous over all but the high current density edge of the current density range.

*Example 7*

Phenylpropionic amide in the amount of 0.2 g./l. was added to the standard tin-nickel bath in a small laboratory tank. A copper-plated zinc die cast handle was plated at approximately 2.3 amp./sq. dm. for 30 minutes. An average tin-nickel thickness of approximately 23 microns was obtained. The deposit was clear-bright and lustrous.

*Example 8*

Phenylpropionic amide in the amount of 0.1 g./l. was added to the standard tin-nickel bath formulation in a Hull Cell. A smooth brass panel was plated for 10 minutes at an average current density of 2.7 amp./sq. dm., the deposit obtained was clear-bright over the entire current density range.

*Example 9*

The compound 1-(p-aminophenyl)-3-methylpyrazole in the amount of 0.5 g./l. was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 10*

The compound 1-(p-aminophenyl)-3-methylpyrazole in the amount of 0.1 g./l. was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 11*

The compound, stearamidopropyldimethyl-( $\beta$ -hydroxyethyl)-ammonium dihydrogen phosphate in the amount of 0.12 g./l. was added to the standard tin-nickel formula-

tion in a Hull Cell. A smooth brass panel was plated at an average current density of 2.7 amp./sq. dm. for 10 minutes. The tin-nickel deposit was clear-bright over the entire panel.

*Example 12*

10 The compound, stearamidopropyldimethyl-( $\beta$ -hydroxyethyl)ammonium dihydrogen phosphate, in the amount of 0.04 g./l. was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 13*

15 The compound 1,5-diphenylcarbohydrazide in the amount of 0.4 g./l. was added to the standard tin-nickel formulation in a Hull Cell. A smooth brass panel was plated at an average current density of 2.7 amp./sq. dm. for 10 minutes. The tin-nickel deposit was hazy-bright 20 over the entire panel.

*Example 14*

25 The compound 1,5-diphenylcarbohydrazide in the amount of 0.10 g./l. was added to the standard tin-nickel formulation in a Hull Cell. A smooth brass panel was plated at an average current density of 2.7 amp./sq. dm. for 10 minutes. The tin-nickel deposit was hazy-bright over the entire panel.

*Example 15*

30 The compound, phosphoric acid ( $H_3PO_4$ ), in the amount of 11 g./l. was added to the standard tin-nickel formulation in a Hull Cell. A smooth brass panel was plated at an average current density of 2.7 amp./sq. dm. 35 for 10 minutes. The tin-nickel deposit was clear-bright over the area of the panel below about 3 amp./sq. dm. and hazy-bright on areas above about 3 amp./sq. dm.

*Example 16*

40 The compound, phosphoric acid ( $H_3PO_4$ ), in the amount of 6 g./l. was added to the standard tin-nickel formulation in a Hull Cell. A smooth brass panel was plated at an average current density of 2.7 amp./sq. dm. for 10 minutes. The tin-nickel deposit was hazy-bright over the entire panel.

*Example 17*

45 The compound, phosphoric acid ( $H_3PO_4$ ), in the amount of 0.6 g./l. was added to the standard tin-nickel formulation in a Hull Cell. A smooth brass panel was plated at an average current density of 2.7 amp./sq. dm. 50 for 10 minutes. The tin-nickel deposit was hazy-bright over the entire panel.

*Example 18*

55 A combination of phenylpropionic acid, 0.08 g./l., and stearamidopropyldimethyl- ( $\beta$ -hydroxyethyl)ammonium hydrogen phosphate, 0.003 g./l., was added to the standard tin-nickel formulation in a Hull Cell. A smooth brass panel was plated at an average current density of 2.7 amp./sq. dm. 60 for 10 minutes. The tin-nickel deposit was clear-bright over the entire panel.

*Example 19*

65 A combination of stearamidopropyldimethyl-( $\beta$ -hydroxyethyl)ammonium dihydrogen phosphate, 0.12 g./l. and phosphoric acid, 1.8 g./l. was added to the standard tin-nickel formulation in a Hull Cell. A smooth brass panel was plated at an average current density of 2.7 amp./sq. dm. for 10 minutes. The tin-nickel deposit 70 was clear-bright over the entire panel.

*Example 20*

A combination of phenylpropionic acid, 0.04 g./l. and phosphoric acid, 0.6 g./l., was added to the standard tin-nickel formulation in a Hull Cell. A smooth brass

panel was plated at an average current density of 2.7 amp./sq. dm. for 10 minutes. The tin-nickel deposit was clear-bright over the entire panel.

*Example 21*

A combination of phenylpropionic amide, 0.06 g./l. and phosphoric acid, 1 g./l., was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 22*

A combination of triaminotriphenyl methane, 0.02 g./l., and phosphoric acid, 0.5 g./l., was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 23*

A combination of 1-(p-aminophenyl)-3-methylpyrazole, 0.1 g./l., and phosphoric acid, 0.8 g./l., was added to the standard tin-nickel formulation in a Hull Cell. A smooth brass panel was plated at an average current density of 2.7 amp./sq. dm. for 10 minutes. The tin-nickel deposit was clear-bright over the entire panel.

*Example 24*

A combination of 1,5-diphenylcarbohydrazide, 0.1 g./l., and phosphoric acid, 2.0 g./l. was added to the standard tin-nickel formulation in a Hull Cell. A smooth brass panel was plated at an average current density of

2.7 amp./sq. dm. for 10 minutes. The tin-nickel deposit was hazy-bright over the entire panel.

Similar lustrous and bright deposits are obtained using the noted additives with other acid baths, such as Bath 5 1 of Table II and the all-chloride bath formulation, at pH values below 1. The tin-nickel electrodeposits obtained from the "bright" baths were strongly oriented in the 300 plane. Utilizing these bright baths, it is possible to electrodeposit bright tin-nickel directly on most 10 basis metals including steel, copper and copper alloys, tin, nickel and nickel alloys, etc. Conventional cleaning of the basis metal prior to electrodeposition should be practiced. The use of a bronze or copper undercoat on some basis metals, particularly those electrochemically 15 active in acid baths, is preferred.

As many embodiments of this invention may be made without departing from the spirit and scope thereof, it is to be understood that the invention includes all such 20 modifications and variations as come within the scope 20 of the appended claim.

We claim:

A composite metal article comprising a basis metal having a surface deposit of a lustrous bright tin-nickel 25 alloy with layering strongly oriented in the 300 plane.

**References Cited by the Examiner**

**UNITED STATES PATENTS**

|           |         |        |        |
|-----------|---------|--------|--------|
| 2,654,703 | 10/1953 | Brown  | 204-43 |
| 2,748,086 | 5/1956  | Faust  | 204-43 |
| 2,926,124 | 2/1960  | Taylor | 204-43 |

HYLAND BIZOT, Primary Examiner.